# EUROPEAN PATENT SPECIFICATION

(11) **EP 3 027 824 B1**
(45) Date of publication and mention of the grant of the patent: **17.03.2021**
(21) Application number: 14758666.3
(22) Date of filing: 24.07.2014
(51) Int. Cl.: E04F 13/16, E04F 15/10

(54) **FLEXIBLE PANEL AND METHOD OF PRODUCTION**
FLEXIBLE PLATTE UND VERFAHREN ZUR HERSTELLUNG
PANNEAU FLEXIBLE ET PROCÉDÉ DE PRODUCTION

(30) Priority: 29.07.2013 IT AR20130029
(43) Date of publication of application: 08.06.2016
(73) Proprietor: Reverberi, Ezio, 58015 Orbetello (IT)
(72) Inventor: Reverberi, Ezio, 58015 Orbetello (IT)
(74) Representative: Petraz, Davide Luigi
(86) International application number: PCT/IB2014/063385
(87) International publication number: WO 2015/015380

(56) References cited:
- EP-A1- 2 586 814
- US-B1- 7 125 601

## Description

### FIELD OF THE INVENTION

The present invention concerns a flexible panel and a corresponding method of production, which constitutes an unusual product, innovative because of the composition of the material and its possible uses, and a method that allows to transform a flexible substrate, such as a soft fabric, of vegetable origin such as for example jute or cotton, or other, or synthetic, inorganic or artificial, or a piece of hide or a sheet of metal, in particular aluminum, possibly also a sheet of self-adhesive aluminum, into a panel or sheet, comparable for example to a robust hide or cloth, consisting of stones or metals, which will be hard but at the same time flexible so as to be able to adapt to cover every type of surface, object or shape.

### BACKGROUND OF THE INVENTION

It is known that hides have an ancient tradition of tanning, and likewise fabrics an ancient tradition of dyeing: these consolidated traditions certainly make these materials very beautiful and soft, with an almost infinite range of materials, colors and textures.

However it is equally well known that the methods for working the fabrics and the hides are extremely polluting for the environment: the dyeing vats for animal or vegetable fabrics require expensive purification plants which often are not able to completely eliminate the pollution of the water, and the hot processes produce steam and carbon nano-particles which are released into the atmosphere.

It is also known that, in building restorations, particularly in old city centers, materials such as stone, marble and handmade terracotta are almost excluded because of their considerable weight and thickness: if they were required, it would be necessary to demolish old floors and coverings.

Currently, tiles or slabs which are not very thick can be found on the market, but these new tiles are fragile and subject to breakage or chipping during work on site.

It is also known that laying traditional slabs and tiles can have disadvantages connected to the fact that traditional slabs or tiles are rigid and not very adaptable to the many different shapes that exist in the buildings being restored; in the state of the art, the tile layer is therefore obliged to cut the tiles or adapt the walls on site.

These cuts are carried out with abrasive disc millers which produce both noise and dust, as well as entailing a lot of working time for the craftsman.

The traditional methods of laying tiles or slabs also have the disadvantage that they need long working times and consequently entail delays in delivering the buildings for use which, if they are for commercial or hotel use, affect the cost of restructuring and entail loss of earnings.

To avoid direct and indirect costs and to obtain a considerable reduction in costs of laying the floors, solutions are typically used which are less thick and weight, such as plastic laminates, PVC slabs, linoleum.

These materials, which are not at all thick or heavy, have the advantage that they are easily layable over previous floorings without having to demolish them, but they are undoubtedly impersonal, flat and slippery, with the tendency to deteriorate over time without realistic possibilities of restoring them.

Another material which is not very thick or heavy and easy to lay is carpet but, as is known, this material is not very satisfactory because of its well known retention of dirt, because it is difficult and costly to keep clean and so it is not hygienic for living areas.

Other solutions currently on the market are self-leveling resins or resins spread on site.

These solutions have shown their limitations, acceptable only in industrial flooring, since they are conditioned by the many difficulties in obtaining a good result in laying them, both because it is difficult to find skilled personnel to apply them, and because the environmental conditions need to be perfect, and also because the many coats to be applied take a long time to dry, but which are necessary to obtain a professional finish; consequently these applications are very costly when finally installed.

EP2586814 A1 discloses a self-crosslinking polyhydroxy polyurethane resin, that can be used to make products, such as imitation leather, a skin material for car interior or home electric appliance component, or weather strip to prevent wind or rain from penetrating through gap of a door.

Document EP-A-0.562.282 describes a water-based varnish to make covering films for furnishing elements made of wood, polyester, polyurethane, polyacrylic, polyepoxides, metal, or covered with a different water-based varnish. The water-based varnish of EP-A-0.562.282 has high resistance to chemical agents and to abrasion, and has an esthetic appearance similar to that of solvent-based varnishes. This varnish provides a mixture of a first component that consists of water-based dispersions of acrylic and urethane polymers and a second component that consists of a liquid poly-isocyanide compound as such, or in a solution with ethylacetate. The varnish provides to use silica oxide as filler, to confer for example hardness, rigidity and resistance to abrasion. In EP-A-0.562.282, the poly-isocyanide is used to reticulate the acrylic-urethane polymer material, and therefore has the properties of hardness, rigidity and resistance to abrasion of reticulated polyurethane bi-component systems, similar to solvent-based systems; it therefore does not have any properties of flexibility such as to be adaptable and shapeable to cover any type of surface, object or shape.

Document GB-A-2.429.419 describes a hydrophobic covering and a hydrophylic covering applied on respective surfaces of a material for an anti-collapsible construction, in particular a fibrous panel for ceilings, in particular for sound-proofing. This solution therefore describes a rigid and structured panel, commonly used suspended to the ceiling for sound-proofing, absolutely unsuitable for covering every type of surface, object or shape.

One purpose of the present invention is to overcome the shortcomings of the state of the art, which provide to consolidate, protect and/or finish the surfaces of materials of already existing articles such as wood, sheet metals, metals and others, proposing the possibility to make a new, intrinsic and completely innovative material, consisting of the association of mineral raw materials, such as stones or metals, in a homogenous compound, in the form of a flexible panel, and a method of production, which represent advantageous alternatives to hides or flexible cloths used in the production of leather goods, luggage or upholstery that can be used without the need for polluting processes or that consume fossil fuels.

Another purpose is to supply a flexible panel and a method of production that represent advantageous alternative solutions to traditional stone materials such as terracotta, stone or marble in building restoration, where it is very important to prevent the demolition of old floorings and coverings, without needing to use materials of a lesser thickness and weight, without quality and personalization, as happens with plastic laminates, thin parquet and vinyl flooring.

The Applicant has devised, tested and embodied the present invention to overcome the shortcomings of the state of the art and to obtain these and other purposes and advantages.

Unless otherwise defined, all the technical and scientific terms used here and hereafter have the same meaning as commonly understood by a person with ordinary experience in the field of the art to which the present invention belongs. Even if methods and materials similar or equivalent to those described here can be used in practice and in the trials of the present invention, the methods and materials are described hereafter as an example. In the event of conflict, the present application shall prevail, including its definitions. The materials, methods and examples have a purely illustrative purpose and shall not be understood restrictively.

### SUMMARY OF THE INVENTION

The present invention is set forth and characterized in the independent claims, while the dependent claims describe other characteristics of the invention or variants to the main inventive idea.

In accordance with the above purposes, forms of embodiment described here concern a cold processed flexible substrate, at least partly covered or impregnated with a dispersion of water-based aliphatic resin in which granules of stone or mineral material are homogeneously distributed, wherein said dispersion of water-based aliphatic resin comprises: -one or more compounds chosen from a group comprising polyurethane compounds:-one or more compounds chosen from a group comprising acrylic compounds: and-one or more compounds chosen from a group comprising styrene compounds: wherein said stone or mineral material is chosen from a group comprising terracotta, stone, marble, crystals, quartzes, metals in general, in particular bronze, steel or iron, wherein in the case of terracotta, the latter has a grain size from 0.3 mm to 1 mm and the terracotta and the dispersion of water-based aliphatic resin are provided in a ratio of 1 part in weight of dispersion of aliphatic resin and 3 parts in weight of terracotta: or, in the case of marble or quartz, the latter have a grain size between 0 µm and 160 µm (micron), or between 0 µm (micron) and 50 µm (micron), or again between 0 µm (micron) and 45 µm (micron): or again, in the case of bronze, the latter has a grain size of 100 mesh or 200 mesh and the bronze and the dispersion of water-based aliphatic resin are provided in a ratio of 1 part in weight of dispersion of aliphatic resin and 5 parts in weight in bronze at 100 mesh, or 1 part in weight of dispersion of aliphatic resin and 4 parts in weight of bronze at 200 mesh, such that the stone or mineral material compound and its texture can be felt and not only seen.

According to possible implementations, the flexible substrate can be chosen from: a length of fabric or hide or a sheet of metal, in particular aluminum for example, possibly also a sheet of self-adhesive metal, in particular a sheet of self-adhesive aluminum.

With the present invention a flexible panel is obtained that can be an innovative hide or cloth or sheet of metal consisting of a flexible substrate, for example a natural vegetable fabric, hide or sheet of metal, in particular aluminum, reinforced with particles of stones, marble, terracotta, crystals, various metals; it is hard but malleable, adaptable to cover every type of surface, object or shape, water-proof, stain-proof and fire-proof.

In accordance with the present description, the fabric can be formed from fibers of natural origin, such as vegetable, animal or mineral, or techno-fibers, such as artificial, synthetic or inorganic fibers.

In accordance with the present description, natural fibers usable in forms of embodiment can be vegetable fibers, chosen for example from a group comprising: cotton, linen, hemp, jute, ramie (or nettle yarn), sisal, coconut, Spanish broom, hibiscus, straw, bamboo.

In accordance with the present description, natural fibers usable in forms of embodiment can be animal fibers chosen for example from a group comprising: wool, hair, silk, horsehair, fine linen.

In accordance with the present description, natural fibers usable in forms of embodiment can be mineral fibers chosen for example from a group comprising: asbestos, metal wires, glass wool.

In accordance with the present description, synthetic fibers usable in forms of embodiment can be chosen from a group comprising: acrylic, modacrylic (acrylic modified to be flame-proof), polyamide (nylon), polyester, polypropylene, polyethylene, vinyl chloride, polyurethane (elastam), Teflon (Gore-Tex), aramid (Kevlar).

In accordance with the present description, inorganic fibers usable in forms of embodiment can be chosen from a group comprising: textile glass, carbon fibers, basalt, metal fibers (copper, silver, gold, steel), metalized fibers.

In accordance with the present description, artificial fibers usable in forms of embodiment can be chosen from a group comprising: rayon, modal, cupro, acetate, triacetate, lyocell, rubber or caoutchouc, viscous or artificial silk.

The present invention also concerns a method for the production of a flexible panel, which comprises at least the following steps:
- making available a quantity of granules of stone or mineral material in dry form;
- making available a quantity of a dispersion of water-based aliphatic resin;
- mixing and homogenizing together by stirring the dispersion of water-based aliphatic resin and the granules of stone or mineral material, obtaining a homogeneous mixture;
- applying the homogenous mixture to a flexible substrate, such as for example a length of cloth or hide or a sheet of metal, in particular aluminum for example, possibly even a sheet of self-adhesive aluminum;
- completely drying the flexible substrate on which the homogeneous mixture has been applied;
- trimming to size the flexible substrate associated to the homogeneous mixture and dried, so as to obtain the flexible panel.

In some forms of embodiment, the homogeneous mixture can be applied to the flexible substrate by means of one or more of the following operations:
- completely immersing the flexible substrate in the homogeneous mixture;
- distributing the homogeneous mixture on one or both sides of the flexible substrate by means of spreading or using a spatula;
- applying, by means of spraying, the homogeneous mixture on one or both sides of the flexible substrate.

The choice of one or the other of these operations can be determined by the typical absorption of the substrate material. For example, if the substrate material is highly absorbent, the immersion system can be used, if the substrate material is averagely absorbent the mixture can be spread or applied using a spatula, while if the substrate material is non-absorbent the mixture can be sprayed.

Furthermore, the present invention also concerns a kit for the application of a flexible panel as described above, comprising:
- a flexible panel in accordance with the present description,
- at least a container containing a homogeneous mixture of a dispersion of water-based aliphatic resin and granules of stone or mineral material;
- an elastic glue, free of solvents and cement compounds.

In accordance with the present description, the object of the present invention is characterized in that it is a new, unusual and very beautiful product from both an esthetic and material point of view, consisting of granules of real stone, marble, crystals, metals, possibly also precious metals, which, through a cold production process transforms soft and delicate fabrics such as cotton or jute or others, into a strong material or hide, hard but at the same time flexible, malleable, workable with scissors and stitches, highly resistant to scratches, unalterable by water, resistant to penetration by stains, fire-proof, restorable over time; with these properties it is safe to use in various environments, adapting to every architectural element, such as stairs, coverings, furniture, furnishings, both in the building trade and in the shipbuilding, aeronautical and railway industries. The friction coefficients which come from using the invention in floors and stairs are higher than 0.40 µ and therefore are in conformity with the provisions of the Italian Ministerial Decree n. 236/89 art. 8.2.2, and the most rigorous anti-slip safety regulations in Europe and the USA.

The invention is characterized by the choice of the granulometric scales which vary in relation to the materials used to make the invention, and by way of non-restrictive example, we shall now give some cases: the grain size or granulometric distribution used for the production of handmade terracotta is comprised of grains from 0.3 mm to 1 mm, while the grain size of marble or quartzes can be considered in a curve that can be determined between 0 µm (micron) - 45 µm (micron), or from 0 µm (micron) to 160 µm (micron); to make white marble of the Carrara type very fine grain sizes are used from 0 µm to 50 µm.

In accordance with possible forms of embodiment, the invention is characterized by the fact that the choices of the grain size are determined in a preliminary step for each type of stone or metal material in technical files which will be made available to the person in charge of production. The technical files will be available together with the sample made, with a note of the grain size used.

In accordance with possible forms of embodiment, the invention is characterized by the determination of the proportions of water-based aliphatic resins with respect to the granules, which are provided in a ratio which varies depending on the hardness and simultaneous malleability to be obtained. The ratios are determined during the production planning step and the corresponding values will be shown in the production files, as described above.

The invention is characterized by the determination of the proportions of the compound of resins and granules as described above; by way of non-restrictive example, we shall now give some cases: handmade terracotta: ratio of 1 (one) part in weight of the consolidating compound and 3 (three) parts of terracotta granules with a granulometric curve from 0 mm to 1 mm; bronze: ratio of 1 (one) part of the consolidating compound and 5 (five) parts of bronze granules of 100 mesh, while the parts of bronze will be 4 (four) if the grains are 200 mesh.

In accordance with possible forms of embodiment, the invention is characterized for its different and variable proportions which, as shown above, differ depending on the grain size and absorbency of the mineral involved in the production, on the hardness, malleability and texture to be conferred on the finished product of the invention. These proportions, even if indicated as a non-restrictive example, cannot be determined in any other way than on the basis of tests carried out concurrently to the production plan, with specific production tables being drawn up where the specifications will be indicated.

In accordance with possible forms of embodiment, the invention is characterized by the production steps which provide to mix the compound of water-based aliphatic resins with a stirrer with helical impellers at a low number of revs, to pour the compound into a whisk or blade stirrer and to introduce the granules, stirring the compound at low and average number of revs to obtain a homogeneous fluid mortar.

In possible forms of embodiment, the introduction of the fluid mortar is introduced into non-stick silicone rubber trays of the size provided for the production.

In accordance with possible forms of embodiment, the invention can provide to immerse the flexible substrate, such as for example a length of cloth, fabric or hide or sheet of metal, in particular aluminum, possibly even a sheet of self-adhesive metal, in particular a sheet of self-adhesive aluminum, of a thickness which can vary from 0.5 mm to 10 mm, in particular from 1 mm to 8 mm, depending on the result to be obtained; to extract the fabric with suitable pliers and to position the fabrics on a plane of silicone rubber or nylon made anti-adherent; to dry at room temperature of no less than 15°C and with humidity no higher than 50%; to sand, de-powder, and apply/impregnate with a flame-proof liquid; to obtain a stain-resistant protection, and to trim the pieces; to preserve them on a ventilated shelf and then to pack them in cardboard boxes for commercial delivery.

In other forms of embodiment, the invention provides to distribute, spread, to apply with a spatula or spray the fluid and homogeneous mortar on one or both sides of the flexible substrate.

In accordance with possible forms of embodiment, the invention is characterized by its hardness yet simultaneous malleability, flexibility and deformability, which can allow it to bend by as much as 100° in the solid mass of the fabric, and not only in the free gaps as happens for other articles laid on a mesh.

In accordance with possible forms of embodiment, the invention is characterized by the fact that it is possible to mix together materials which are very different from each other, such as stones, terracotta, metals, possibly even precious metals, combinable with each other as desired. The invention thus differs from yarns that consist of only one element whether it is organic or mineral.

These and other aspects, characteristics and advantages of the present disclosure will be better understood with reference to the following description, drawings and attached claims. The drawings, which are integrated and form part of the present description, show some forms of embodiment of the present invention, and together with the description, are intended to describe the principles of the disclosure.

The various aspects and characteristics described in the present description can be applied individually where possible. These individual aspects, for example aspects and characteristics described in the attached dependent claims, can be the object of divisional applications.

It is understood that any aspect or characteristic that is discovered, during the patenting process, to be already known, shall not be claimed and shall be the object of a disclaimer.

### BRIEF DESCRIPTION OF THE DRAWINGS

These and other characteristics of the present invention will become apparent from the following description of some forms of embodiment, given as a non-restrictive example with reference to the attached drawings wherein:
- fig. 1 is a representation of a natural vegetable fabric usable in forms of embodiment described here;
- fig. 2 is a representation of forms of embodiment described here with granules of terracotta;
- fig. 3 is a representation of forms of embodiment described here with bronze;
- fig. 4 is a representation of a tray usable in forms of embodiment described here;
- fig. 5 is a representation of a whisk mixer usable in forms of embodiment described here;
- fig. 6 is a representation of a blade mixer usable in forms of embodiment described here.

### DESCRIPTION OF THE INVENTION

We shall now refer in detail to the various forms of embodiment of the present invention, of which one or more examples are shown in the attached drawing. Each example is supplied by way of illustration of the invention and shall not be understood as a limitation thereof. For example, the characteristics shown or described insomuch as they are part of one form of embodiment can be adopted on, or in association with, other forms of embodiment to produce another form of embodiment. It is understood that the present invention shall include all such modifications and variants.

Forms of embodiment described here concern the cold transformation of a flexible substrate, such as for example a length of fabric (fig. 1) or a fabric of woven fibers, of natural origin, in particular vegetable, or synthetic, inorganic or artificial, or a piece of hide or a sheet of metal, in particular aluminum, into a flexible panel according to the invention, which represents an innovative "mineral hide or fabric", hard but flexible, adaptable and workable both by cutting with scissors and with stitching, with fire-proof properties, unaffected by water and impenetrable by stains, even oil or grease stains.

The invention can be realized by incorporating into the mass of the flexible substrate, such as fabric, natural or synthetic, inorganic or artificial, or piece of hide or sheet of metal, in particular aluminum, the granules of materials chosen for the type of production, for example terracotta, stone, metal, by immersion in a homogeneous mixture in which the granules and a dispersion of a water-based aliphatic resin are present, that is, a compound of water-based aliphatic resins, without solvents and hydraulic binders that will consolidate in a cold process, at room temperature, without having recourse to ovens for baking them.

In other variants, it is possible to distribute, in particular by spreading or using a spatula, a homogeneous mixture of the citied granules and the dispersion of water-based aliphatic resin on one or both sides of the flexible substrate.

In yet other variants, it is possible to apply the homogeneous mixture on one or both sides of the flexible substrate by spraying. To this end, spraying apparatuses can be used, for example, able to spray mixtures that include inert components in granule form, for example with a grain size of up to 3 mm.

The choice of which of the variants to use can depend for example on the viscosity of the homogeneous mixture and/or the nature or type of flexible substrate on which the homogeneous mixture is applied.

In accordance with the forms of embodiment described here, the resins can be balanced in quantity and quality so as to produce a hardening comparable to the hardness of the mineral element chosen for the compound, at the same time keeping the malleability typical of fabrics.

The material appearance of the invention can be that of the mineral of which it consists, and therefore there are numerous variables that can be obtained, both due to the nature of the mineral compound and its texture, which can be felt and not only seen, as happens instead with materials reproduced using photographic and typographic processes.

As well as its naturalness and the variety of its material appearance, the invention is also characterized by its waterproof properties, and for this reason it is perfectly compatible for use in exteriors; the hide or fabric according to the present invention does not absorb also elements of dirt carried by oil or grease and, if it comes into contact with fire, it carbonizes without a flame and without giving off toxic fumes.

Given the totally innovative characteristics and the beauty of the material, the present invention can also be advantageously used in many fields of manufacturing, such as leather goods, the production of bags, suitcases, trunks and similar, clothing, footwear, gold or jewelry, or coverings for furniture, in furnishing, stairs, columns, floors and various architectural components.

Its characteristics of lightness, thinness, impenetrability by water and grease, and resistance to fire, can also meet important requirements in the field of finishing in interiors and exteriors in the building trade, shipbuilding, interiors in the aeronautical industry and suchlike.

The invention allows to lay, over the old coverings, quality materials such as natural stones, handmade terracotta or precious metals which in addition to low thickness and weight, have the added value of the quality of the materials, personalized finish and, thanks to the invention, the malleability needed to adapt to every type of shape and surface.

The invention is an innovative product similar to hides and fabrics, but with the advantage that it has a high esthetic quality and material, and a strength given by the mineral materials of which it is made, together with the malleability which allows a very varied use as a covering material.

To these advantages must be added its resistance to water, impenetrability by dirt and grease, high resistance to scratching, and ease of restoration: these qualities make the invention an innovative "mineral hide", usable in the field of leather goods, suitcases, coverings for furniture and furnishings, and in various fields of industrial production.

In addition to the above, it should also be emphasized that the invention is easy to produce, the whole cycle and the final product are environmentally friendly, so that the invention can be industrialized economically.

With regard to its use in the field of leather goods, suitcases and upholstery, we stress that the invention is produced with a cold process, without producing waste water and, since it is a cold production, without emission of fumes and particulate into the atmosphere.

The incorporation of the mineral granules in the mass of the flexible substrate, for example of the fabrics or hide or sheet of metal, in particular aluminum, is achieved through a process of consolidation without baking in ovens, totally without solvents, without consuming any fossil fuels and therefore in an environmentally sustainable manner.

With the invention it is possible to make flexible panels similar to fabrics or hides of extraordinary strength and esthetic quality, both to sight and touch, comparable to the skins of reptiles such as crocodile, python and other animals, but with the present invention it is not necessary to kill animals.

On the contrary, the fabrics and compounds according to the invention are made of recycled materials, discarded because of breakages or unsold merchandise lying in the yards.

The granules are obtained by granulating with suitable hammer mills, they are de-powdered and progressively sieved, with the intention of obtaining determinate ranges of grain sizes.

These are the raw materials used to make the invention, for which we exclude the re-use of trash, whatever its nature.

Working the invention to make the models or for various coverings can be done with traditional cutting and stitching systems, as happens for hides or fabrics with a certain consistency.

The invention does not absorb water or dirt and, in the event of fire, carbonizes without producing flames or toxic vapors: this gives a considerable improvement in performance compared with vegetable and animal fabrics which absorb water and dirt and almost always produce flames when they burn.

With regard to use in the building trade, various shipbuilding, coverings, architectural components, furniture and furnishing, it is stressed that the present invention allows to finish materials such as stone, handmade terracotta (fig. 2), metal materials like bronze (fig. 3), steel, and iron, with thin and light materials, without having to renounce beauty and architectural value.

The invention also gives a big advantage over laying traditional slabs and tiles, in terms of flexibility in preparation and laying, and also shorter times for production and laying. The same advantage can be found in shipbuilding, aeronautics and train building where, in addition to its lightness and thinness, the invention's qualities of anti-slip safety, high resistance to penetration by dirt, resistance to wetting and inertia to fire are greatly appreciated.

Another considerable advantage over products available today is the reduced working time and absolute precision, since the flexible panels made with the invention can be cut with normal work scissors, thus adapting them precisely to every shape, silently, without producing dust and hence in total safety for the operator, without inconvenience for neighbors and without damage to the surrounding environment.

In other words, the panels according to the present invention, although they consist of materials of considerable value like precious stones, handmade terracotta, marble and metal compounds, can be laid quickly, at reduced cost, just as happens for example for laying carpet.

Moreover, the present invention helps to overcome various limits such as:
a) obtaining biocompatible finishings for interiors and exteriors, advantageously formed by vegetable natural products, or synthetic, inorganic or artificial products, preferably biodegradable, and minerals, re-composed with water-based organic binder, without cement binders or volatile organic compounds;
b) it allows to recycle materials that otherwise would be sent for disposal due to breakages, or to recycle unsold merchandise, which occupies and unnecessarily obstructs the yards of factories and furnaces, spoiling the environment;
c) it limits the extraction of quarry material or cooking clay, thus saving material and limiting the disfigurement of the territory, with consequent elimination of CO₂ emissions and other greenhouse gases.

### DESCRIPTION OF SOME FORMS OF EMBODIMENT

We shall now describe some forms of embodiment of a method for producing a flexible panel according to the present description, including the following operating steps:
1. The granules of the material to be produced (e.g. terracotta, Serena stone, marble, bronze and others) are prepared, chosen in the most suitable particle size for what is to be produced. The grain size will vary depending on the type of granules to be produced, on the minimum and maximum grain size scale available, on the absorption that the nature of the material and its granulometric composition determine. By way of non-restrictive example, we report the grain size used for the production of handmade terracotta which is sieved and de-powdered with grains from 0.3 mm to 1 mm, while the grain size of marble or quartzes can be considered in a curve between 0 µm (micron) and 45 µm (micron), or between 0 µm (micron) and 160 µm (micron); for marble very fine grain sizes can be achieved, from 0 µm (micron) to 50 µm (micron).
2. On the side, a dispersion of water-based aliphatic resin is prepared, formulated for example with polyurethane and/or acrylic and/or styrene compounds, and other consolidating and fire-proofing compounds, adequately balanced so as to recompose the properties of hardness of the stone or metal, and the flexibility typical of a hide or a textile covering. The ratio of the components of the dispersion of water-based aliphatic resins will vary depending on the type of mineral material to be produced, as well as the level of malleability to be obtained.
3. For industrial production, the variable data given in points 1 and 2 will be determined in advance and displayed in the corresponding production files, which will be made available to the person in charge of production. The same thing will be established to determine the ratio between the dispersion of water-based aliphatic resins and the granules, divided by type.
4. When the weight of the production to be obtained has been determined, as provided in point 3 above, the following will be determined.
   4.1 The weight of the granules in proportion to the weight of the consolidating dispersion.
   4.2 The grain size curve provided for that production will be chosen, and the dry mixture of the granules will be introduced, all together, into a suitable container.
   4.3 The components of the water-based aliphatic resins, suitably dosed in the ratio established for that production, will be introduced into the tank of an electromechanical stirrer equipped with helical impellers (fig. 5). Then the stirrer will be made to function at a low number of revs.
   4.4 After about 5 minutes stirring, the compound will be poured into another electromechanical mixer with a whisk or blades (fig. 6), into which, lightly stirred, the granules prepared at point 4.2 will be introduced from the container where they had been slowly put.
   4.5 When the whole quantity of the granules has been introduced, the number of revs of the whisk or blade stirrer will be increased; if the stirrer is a whisk stirrer, it will have to be equipped with an oscillating head so as to better homogenize the compound being stirred.
5. When a fluid and well homogenized mortar has thus been obtained (homogeneous mixture of inert materials and dispersion of water-based aliphatic resins), the mortar will be applied to a flexible substrate such as a sheet of fabric or hide or sheet of metal, in particular aluminum, possibly also a sheet of self-adhesive aluminum, in such a way that the substrate is at least partly or completely covered by or impregnated with said mixture.
   5.1 For example, if the substrate is highly absorbent, like a length of fabric, the mortar is poured into a tray-shaped container (fig. 4) made of silicone rubber or nylon or steel, all made anti-adherent. The container will be the same size as the pieces of fabric to be produced. On the tray thus prepared, the flexible substrate will be rested, such as a length of fiber/fabric, for example natural vegetable, or synthetic, inorganic or artificial (fig. 1) which will have a thickness that can vary from 1.00 mm to about 8 mm; the flexible substrate will be immersed and sunk in the mortar formed by the homogeneous mixture of inert materials and the dispersion of water-based aliphatic resins, to be completely covered; then, the flexible substrate, well soaked, will be removed with a suitable pincer, and then rested on a holed plane made of silicone rubber or nylon or steel, suitably treated with an anti-adherent product in an environment at a temperature of not less than 15° C with humidity of not more than 50%.
   5.2 The complete drying of the flexible substrates produced, on which the homogeneous mixture of inert materials and dispersion of water-based aliphatic resins has been applied, will take place in the conditions as described above, after about 24 hours, after which it will be assessed whether the product (flexible panel) esthetically respects the properties of the material to which it refers (e.g. handmade terracotta, bronze and others) and based on this assessment the product will be finished by sanding, de-powdering and application/impregnation in a suitably prepared fireproof liquid.
   5.3 Finally, on the flexible panel obtained the anti-stain protection will be applied, consisting of a dispersion of specific water-based aliphatic resins or a special water-based anti-stain wax; these protections will be applied using a microfiber roller; it will take about 4 or 5 hours to dry each coat of protection.
   5.4 When dry, each panel produced will be trimmed to the sizes required, all the same, and then deposited on an open shelf, well ventilated, where each type produced will be stored, divided by type of material, size and shape, and then packaged in cardboard boxes to be sent to its final destination.
   5.5 Together with the flexible panel produced, buckets of polyethylene will be packaged, containing the same compound used to produce the mortar for the sheets, so that the mortar can be supplied together with the sheets so that finishing and personalization can be carried out when the flexible panel is installed.
6. For the application of the panels according to the present invention two types of glue will be produced, extremely elastic, without solvents and cement compounds: a thin water-based glue for gluing in the gift and fancy goods sector, furnishing, furniture, leather goods and other similar applications, and a thick glue loaded with very fine inert materials, but also without solvents and cement compounds, to be used for gluing the invention to floors, stairs and other architectural elements.
7. For use in the field of leather goods and other articles, the methods for using the lengths of fabric or hide according to the present invention will be decided by each purchaser/user, who will use the best working techniques depending on his own product, maintaining the proper confidentiality thereof.
8. In the field of coverings in the building trade, and shipbuilding in general, the requirements are different and the choice of the application systems depends on the situations found by the person doing the laying, personalizing the finishing with spatula effects, colors, shades of color on color, which is the most precious finishing characteristic of the invention, with which it will be possible to obtain highly prestigious works, personalized, characterized by different textures, never the same, unlike what happens with products made using molds.

As a variant to point 5.1, depending on the type of flexible substrate, the fluid and homogenized mortar formed by the homogeneous mixture of inert materials and dispersion of water-based aliphatic resins may be spread or applied with a spatula on one or both sides of the flexible substrate (for example if the substrate is averagely absorbent), or again, the mortar can be sprayed on one or both sides of the flexible substrate (for example if the substrate is not absorbent).

It should be noted here that a flexible substrate as used in the forms of embodiment described here can be at least one element selected from the group consisting of: a length of fabric or fiber, natural, synthetic, or artificial, mineral, intending both warp and weave fabric, woven fabric, or made with other techniques, both non-woven fabric, or sheets or lengths of hide, intending both natural hide and imitation or synthetic hide, or sheets of metal, in particular thin sheets of metal, for example sheets of aluminum, possibly also sheets of self-adhesive metal, in particular sheets of self-adhesive aluminum, and similar articles.

It is also clear that, although the present invention has been described with reference to some specific examples, a person of skill in the art shall certainly be able to achieve many other equivalent forms of flexible panel and method to make it, having the characteristics as set forth in the claims and hence all coming within the field of protection defined thereby.

## Claims

1. Flexible panel, **characterized in that** it comprises a cold processed flexible substrate, at least partly covered or impregnated with a dispersion of water-based aliphatic resin in which granules of stone or mineral material are homogeneously distributed, wherein said dispersion of water-based aliphatic resin comprises:
- one or more compounds chosen from a group comprising polyurethane compounds;
- one or more compounds chosen from a group comprising acrylic compounds; and
- one or more compounds chosen from a group comprising styrene compounds; wherein said stone or mineral material is chosen from a group comprising terracotta, stone, marble, crystals, quartzes, metals in general, in particular bronze, steel or iron, wherein in the case of terracotta, the latter has a grain size from 0.3 mm to 1 mm and the terracotta and the dispersion of water-based aliphatic resin are provided in a ratio of 1 part in weight of dispersion of aliphatic resin and 3 parts in weight of terracotta; or, in the case of marble or quartz, the latter have a grain size between 0 µm (micron) and 160 µm (micron), or between 0 µm (micron) and 50 µm (micron), or again between 0 µm (micron) and 45 µm (micron); or again, in the case of bronze, the latter has a grain size of 100 mesh or 200 mesh and the bronze and the dispersion of water-based aliphatic resin are provided in a ratio of 1 part in weight of dispersion of aliphatic resin and 5 parts in weight in bronze at 100 mesh, or 1 part in weight of dispersion of aliphatic resin and 4 parts in weight of bronze at 200 mesh, such that the stone or mineral material and its texture can be felt and not only seen.

2. Flexible panel, **characterized in that** said flexible substrate is chosen from a group comprising: a length of fabric or hide or a sheet of metal, in particular aluminum.

3. Flexible panel as in claim 1, **characterized in that** the fabric has a base of natural fibers, or techno-fibers.

4. Flexible panel as in any claim hereinbefore, **characterized in that** said dispersion of water-based aliphatic resin comprises one or more compounds chosen from a group comprising consolidating compounds.

5. Flexible panel as in any claim hereinbefore, **characterized in that** it comprises one or more compounds chosen from a group comprising fireproofing compounds.

6. Flexible panel as in claims 4 and 5, **characterized in that** it comprises consolidating compounds and fireproofing compounds.

7. Flexible panel as in any claim hereinbefore, **characterized in that** the flexible substrate has a thickness comprised between 0.5 mm and 10 mm, in particular between 1 mm and 8 mm.

8. Flexible panel as in any claim hereinbefore, for use in the production of leather goods, luggage or upholstery, or for use as covering material in the building or furnishing trades.

9. Method to make a flexible panel, **characterized in that** the method involves a cold processing of a flexible substrate, comprising at least the following steps:
- making available a quantity of granules of stone or mineral material in dry form;
- making available a quantity of a dispersion of water-based aliphatic resin;
- mixing and homogenizing together by stirring the dispersion of water-based aliphatic resin and the granules of stone or mineral material, obtaining a homogeneous mixture;
- applying said homogenous mixture to a flexible substrate;
- completely drying the flexible substrate on which the homogeneous mixture has been applied;
- trimming to size the flexible substrate on which the homogeneous mixture has been applied and dried, so as to obtain said flexible panel;
wherein said dispersion of water-based aliphatic resin comprises:
- one or more compounds chosen from a group comprising polyurethane compounds;
- one or more compounds chosen from a group comprising acrylic compounds; and
- one or more compounds chosen from a group comprising styrene compounds; wherein said stone or mineral material is chosen from a group comprising terracotta, stone, marble, crystals, quartzes, metals in general, in particular bronze, steel or iron, wherein in the case of terracotta, the latter has a grain size from 0.3 mm to 1 mm and the terracotta and the dispersion of water-based aliphatic resin are provided in a ratio of 1 part in weight of dispersion of aliphatic resin and 3 parts in weight of terracotta; or, in the case of marble or quartz, the latter have a grain size between 0 µm (micron) and 160 µm (micron), or between 0 µm (micron) and 50 µm (micron), or again between 0 µm (micron) and 45 µm (micron); or again, in the case of bronze, the latter has a grain size of 100 mesh or 200 mesh and the bronze and the dispersion of water-based aliphatic resin are provided in a ratio of 1 part in weight of dispersion of aliphatic resin and 5 parts in weight in bronze at 100 mesh, or 1 part in weight of dispersion of aliphatic resin and 4 parts in weight of bronze at 200 mesh, such that the stone or mineral material and its texture can be felt and not only seen.

10. Method as in claim 9, **characterized in that** the application of said homogeneous mixture to said flexible substrate occurs by means of one or more, as chosen, of the following operations:
- completely immersing the flexible substrate in the homogeneous mixture;
- distributing said homogeneous mixture on one or both sides of the flexible substrate in particular by spreading or by using a spatula;
- applying, by means of spraying, said homogeneous mixture on one or both sides of the flexible substrate.

11. Method as in claim 9 or 10, **characterized in that,** before trimming to size, it provides to finish the flexible substrate on which the homogeneous mixture has been applied and dried by means of sanding, de-powdering, and application/impregnation in a flame-proof liquid, and to obtain a stain-resistant protection.

12. Method as in claim 9, 10 or 11, **characterized in that** said flexible substrate is chosen from a group comprising: a length of fabric or hide or a sheet of metal, in particular aluminum.

13. Kit comprising:
- a flexible panel as in any claim from 1 to 8;
- at least a container containing a homogeneous mixture of a dispersion of water-based aliphatic resin and granules of stone or mineral material;
- an elastic glue, free of solvents and cement compounds.

## Patentansprüche

1. Flexibles Paneel, **dadurch gekennzeichnet, dass** es ein kaltverarbeitetes flexibles Substrat aufweist, das zumindest teilweise mit einer Dispersion eines aliphatischen Harzes auf Wasserbasis bedeckt oder imprägniert ist, in der Körnchen aus Stein- oder Mineralmaterial homogen verteilt sind, wobei die Dispersion von aliphatischem Harz auf Wasserbasis aufweist:
- eine oder mehr Verbindungen, die aus einer Gruppe ausgewählt sind, die Polyurethanverbindungen aufweist,
- eine oder mehr Verbindungen, die aus einer Gruppe ausgewählt sind, die Acrylverbindungen aufweist, und
- eine oder mehr Verbindungen, die aus einer Gruppe ausgewählt sind, die Styrolverbindungen aufweist,
wobei das Stein- oder Mineralmaterial aus einer Gruppe ausgewählt ist, die Terrakotta, Stein, Marmor, Kristalle, Quarze, Metalle im Allgemeinen, insbesondere Bronze, Stahl oder Eisen aufweist, wobei im Fall von Terrakotta letztere eine Korngröße von 0,3 mm bis 1 mm hat und die Terrakotta und die Dispersion von aliphatischem Harz auf Wasserbasis in einem Verhältnis von 1 Gewichtsteil Dispersion von aliphatischem Harz und 3 Gewichtsteilen Terrakotta vorgesehen sind, oder im Fall von Marmor oder Quarz letztere eine Korngröße zwischen 0 µm (Mikron) und 160 µm (Mikron), oder zwischen 0 µm (Mikron) und 50 µm (Mikron), oder auch zwischen 0 µm (Mikron) und 45 µm (Mikron) haben, oder auch im Fall von Bronze diese eine Korngröße von 100 Mesh oder 200 Mesh hat und die Bronze und die Dispersion von aliphatischem Harz auf Wasserbasis in einem Verhältnis von 1 Gewichtsteil Dispersion von aliphatischem Harz und 5 Gewichtsteilen Bronze bei 100 Mesh oder 1 Gewichtsteil Dispersion von aliphatischem Harz und 4 Gewichtsteilen Bronze bei 200 Mesh vorgesehen sind, so dass das Stein- oder Mineralmaterial und seine Textur fühlbar und nicht nur sichtbar sind.

2. Flexibles Paneel, **dadurch gekennzeichnet, dass** das flexible Substrat aus einer Gruppe ausgewählt ist, die aufweist: eine Stoff- oder Hautbahn oder ein Blech aus Metall, insbesondere Aluminium.

3. Flexibles Paneel gemäß Anspruch 1, **dadurch gekennzeichnet, dass** der Stoff eine Basis aus Naturfasern oder Technofasern hat.

4. Flexibles Paneel gemäß irgendeinem vorhergehenden Anspruch, **dadurch gekennzeichnet, dass** die Dispersion von aliphatischem Harz auf Wasserbasis eine oder mehrere Verbindungen aufweist, die aus einer Gruppe ausgewählt sind, die verfestigende Verbindungen aufweist.

5. Flexibles Paneel gemäß irgendeinem vorhergehenden Anspruch, **dadurch gekennzeichnet, dass** es eine oder mehrere Verbindungen aufweist, die aus einer Gruppe ausgewählt sind, die feuerfeste Verbindungen aufweist.

6. Flexibles Paneel gemäß den Ansprüchen 4 und 5, **dadurch gekennzeichnet, dass** es verfestigende Verbindungen und feuerfeste Verbindungen aufweist.

7. Flexibles Paneel gemäß irgendeinem vorhergehenden Anspruch, **dadurch gekennzeichnet, dass** das flexible Substrat eine Dicke zwischen 0,5 mm und 10 mm, insbesondere zwischen 1 mm und 8 mm, hat.

8. Flexibles Paneel gemäß irgendeinem vorhergehenden Anspruch, zur Verwendung bei der Herstellung von Lederwaren, Gepäck oder Polsterungen oder zur Verwendung als Abdeckmaterial im Bau- oder Einrichtungsgewerbe.

9. Verfahren zur Herstellung eines flexiblen Paneels, **dadurch gekennzeichnet, dass** das Verfahren eine Kaltverarbeitung eines flexiblen Substrats beinhaltet, aufweisend mindestens die folgenden Schritte:
- Bereitstellen einer Menge von Körnchen aus Stein- oder Mineralmaterial in trockener Form,
- Bereitstellen einer Menge einer Dispersion eines aliphatischen Harzes auf Wasserbasis,
- Mischen und Homogenisieren der Dispersion von aliphatischem Harz auf Wasserbasis und der Körnchen aus Stein- oder Mineralmaterial durch Rühren, wodurch ein homogenes Gemisch erhalten wird,
- Aufbringen des homogenen Gemischs auf ein flexibles Substrat,
- vollständiges Trocknen des flexiblen Substrats, auf das das homogene Gemisch aufgebracht wurde,
- Zuschneiden des flexiblen Substrats, auf das das homogene Gemisch aufgebracht und welches getrocknet wurde, um das flexible Paneel zu erhalten,
wobei die Dispersion von aliphatischem Harz auf Wasserbasis aufweist:
- eine oder mehr Verbindungen, die aus einer Gruppe ausgewählt werden, die Polyurethanverbindungen aufweist,
- eine oder mehr Verbindungen, die aus einer Gruppe ausgewählt werden, die Acrylverbindungen aufweist, und
- eine oder mehr Verbindungen, die aus einer Gruppe ausgewählt werden, die Styrolverbindungen aufweist,
wobei das Stein- oder Mineralmaterial aus einer Gruppe ausgewählt wird, die Terrakotta, Stein, Marmor, Kristalle, Quarze, Metalle im Allgemeinen, insbesondere Bronze, Stahl oder Eisen aufweist, wobei im Fall von Terrakotta letztere eine Korngröße von 0,3 mm bis 1 mm hat und die Terrakotta und die Dispersion von aliphatischem Harz auf Wasserbasis in einem Verhältnis von 1 Gewichtsteil Dispersion von aliphatischem Harz und 3 Gewichtsteilen Terrakotta vorgesehen sind, oder im Fall von Marmor oder Quarz, letztere eine Korngröße zwischen 0 µm (Mikron) und 160 µm (Mikron) oder zwischen 0 µm (Mikron) und 50 µm (Mikron) oder auch zwischen 0 µm (Mikron) und 45 µm (Mikron) aufweisen, oder auch im Fall von Bronze diese eine Korngröße von 100 Mesh oder 200 Mesh hat und die Bronze und die Dispersion von aliphatischem Harz auf Wasserbasis in einem Verhältnis von 1 Gewichtsteil Dispersion von aliphatischem Harz und 5 Gewichtsteilen Bronze bei 100 Mesh oder 1 Gewichtsteil Dispersion von aliphatischem Harz und 4 Gewichtsteilen Bronze bei 200 Mesh vorgesehen sind, so dass das Stein- oder Mineralmaterial und seine Textur fühlbar und nicht nur sichtbar sind.

10. Verfahren gemäß Anspruch 9, **dadurch gekennzeichnet, dass** das Aufbringen des homogenen Gemischs auf das flexible Substrat mittels eines oder mehrerer, wie gewählt, der folgenden Vorgänge erfolgt:
- vollständiges Eintauchen des flexiblen Substrats in das homogene Gemisch,
- Verteilen des homogenen Gemischs auf einer oder beiden Seiten des flexiblen Substrats, insbesondere durch Aufstreichen oder durch Verwenden eines Spatels,
- Auftragen des homogenen Gemischs auf eine oder beide Seiten des flexiblen Substrats durch Sprühen.

11. Verfahren gemäß Anspruch 9 oder 10, **dadurch gekennzeichnet, dass** es vor dem Zuschneiden vorsieht, das flexible Substrat, auf das das homogene Gemisch aufgetragen und getrocknet wurde, mittels Schleifens, Entpuderns und Auftragens/Imprägnierens in einer feuerfesten Flüssigkeit fertigzubearbeiten und einen schmutzabweisenden Schutz zu erhalten.

12. Verfahren gemäß Anspruch 9, 10 oder 11, **dadurch gekennzeichnet, dass** das flexible Substrat aus einer Gruppe ausgewählt wird, die aufweist: eine Stoff- oder Hautbahn oder ein Blech aus Metall, insbesondere Aluminium.

13. Kit, aufweisend:
- ein flexibles Paneel gemäß irgendeinem Anspruch von 1 bis 8,
- mindestens einen Behälter, der ein homogenes Gemisch einer Dispersion eines aliphatischen Harzes auf Wasserbasis und Körnchen aus Stein- oder Mineralmaterial enthält,
- einen elastischer Klebstoff, frei von Lösungsmitteln und Zementverbindungen.

## Revendications

1. Panneau flexible, **caractérisé en ce qu'**il comprend un substrat flexible traité à froid, au moins partiellement recouvert ou imprégné d'une dispersion de résine aliphatique à base d'eau dans laquelle des granulés de pierre ou de matière minérale sont distribués de manière homogène, où ladite dispersion de résine aliphatique à base d'eau comprend :
- un ou plusieurs composés choisis dans un groupe comprenant des composés de polyuréthane ;
- un ou plusieurs composés choisis dans un groupe comprenant des composés acryliques ; et
- un ou plusieurs composés choisis dans un groupe comprenant des composés styréniques ;
où ladite pierre ou ladite matière minérale est choisie dans un groupe comprenant la terre cuite, la pierre, le marbre, les cristaux, les quartz, les métaux en général, en particulier le bronze, l'acier ou le fer, où dans le cas de la terre cuite, celle-ci a une granulométrie de 0,3 mm à 1 mm et la terre cuite et la dispersion de résine aliphatique à base d'eau sont fournies dans un rapport de 1 partie en poids de dispersion de résine aliphatique et de 3 parties en poids de terre cuite ; ou dans le cas du marbre ou du quartz, ces derniers ont une granulométrie comprise entre 0 µm (micron) et 160 µm (micron), ou entre 0 µm (micron) et 50 µm (micron), ou encore entre 0 µm (micron) et 45 µm (micron) ; ou encore, dans le cas du bronze, ce dernier a une granulométrie de 100 mesh ou 200 mesh et le bronze et la dispersion de résine aliphatique à base d'eau sont fournis dans un rapport de 1 partie en poids de dispersion de résine aliphatique et 5 parties en poids de bronze à 100 mesh, ou 1 partie en poids de dispersion de résine aliphatique et 4 parties en poids de bronze à 200 mesh, de sorte que la pierre ou la matière minérale et sa texture peuvent être ressentis et non seulement vus.

2. Panneau flexible, **caractérisé en ce que** ledit substrat flexible est choisi dans un groupe comprenant : une longueur de tissu ou de cuir ou une feuille de métal, en particulier d'aluminium.

3. Panneau flexible selon la revendication 1, **caractérisé en ce que** le tissu a une base de fibres naturelles, ou techno-fibres.

4. Panneau flexible selon l'une quelconque des revendications précédentes, **caractérisé en ce que** ladite dispersion de résine aliphatique à base d'eau comprend un ou plusieurs composés choisis dans un groupe comprenant des composés de consolidation.

5. Panneau flexible selon l'une quelconque des revendications précédentes, **caractérisé en ce qu'**il comprend un ou plusieurs composés choisis dans un groupe comprenant des composés ignifugeants.

6. Panneau flexible selon les revendications 4 et 5, **caractérisé en ce qu'**il comprend des composés de consolidation et des composés ignifugeants.

7. Panneau flexible selon l'une quelconque des revendications précédentes, **caractérisé en ce que** le substrat flexible a une épaisseur comprise entre 0,5 mm et 10 mm, en particulier entre 1 mm et 8 mm.

8. Panneau flexible selon l'une quelconque des revendications précédentes, destiné à être utilisé dans la production d'articles en cuir, de bagages ou de rembourrage, ou destiné à être utilisé comme matériau de revêtement dans les métiers du bâtiment ou de l'ameublement.

9. Procédé de fabrication d'un panneau flexible, **caractérisé en ce que** le procédé implique un traitement à froid d'un substrat flexible, comprenant au moins les étapes suivantes :
- la mise à disposition d'une quantité de granulés de pierre ou de matière minérale sous forme sèche ;
- la mise à disposition d'une quantité d'une dispersion de résine aliphatique à base d'eau ;
- le mélange et l'homogénéisation en agitant la dispersion de résine aliphatique à base d'eau et les granulés de pierre ou de matière minérale, pour obtenir un mélange homogène ;
- l'application dudit mélange homogène sur un substrat flexible ;
- le séchage complet du substrat flexible sur lequel le mélange homogène a été appliqué ;
- le rognage pour dimensionner le substrat flexible sur lequel le mélange homogène a été appliqué et séché, de manière à obtenir ledit panneau flexible ;
où ladite dispersion de résine aliphatique à base d'eau comprend :
- un ou plusieurs composés choisis dans un groupe comprenant des composés de polyuréthane ;
- un ou plusieurs composés choisis dans un groupe comprenant des composés acryliques ; et
- un ou plusieurs composés choisis dans un groupe comprenant des composés styréniques ;
où ladite pierre ou ladite matière minérale est choisie dans un groupe comprenant la terre cuite, la pierre, le marbre, les cristaux, les quartz, les métaux en général, en particulier le bronze, l'acier ou le fer, où dans le cas de la terre cuite, celle-ci a une granulométrie de 0,3 mm à 1 mm et la terre cuite et la dispersion de résine aliphatique à base d'eau sont fournies dans un rapport de 1 partie en poids de dispersion de résine aliphatique et de 3 parties en poids de terre cuite ; ou dans le cas du marbre ou du quartz, ces derniers ont une granulométrie comprise entre 0 µm (micron) et 160 µm (micron), ou entre 0 µm (micron) et 50 µm (micron), ou encore entre 0 µm (micron) et 45 µm (micron) ; ou encore, dans le cas du bronze, ce dernier a une granulométrie de 100 mesh ou 200 mesh et le bronze et la dispersion de résine aliphatique à base d'eau sont fournis dans un rapport de 1 partie en poids de dispersion de résine aliphatique et 5 parties en poids de bronze à 100 mesh, ou 1 partie en poids de dispersion de résine aliphatique et 4 parties en poids de bronze à 200 mesh, de sorte que la pierre ou la matière minérale et sa texture peuvent être ressentis et non seulement vus.

10. Procédé selon la revendication 9, **caractérisé en ce que** l'application dudit mélange homogène sur ledit substrat flexible se fait au moyen d'une ou plusieurs, au choix, des opérations suivantes :
- l'immersion complète du substrat flexible dans le mélange homogène ;
- la répartition dudit mélange homogène sur un ou les deux côtés du substrat flexible notamment par étalement ou en utilisant une spatule ;
- l'application, par pulvérisation, dudit mélange homogène sur un côté ou sur les deux côtés du substrat flexible.

11. Procédé selon la revendication 9 ou 10, **caractérisé en ce qu'**il prévoit, avant le rognage sur mesure, de finir le substrat flexible sur lequel le mélange homogène a été appliqué et séché au moyen d'un ponçage, d'un dépoussiérage et d'une application/imprégnation dans un liquide ignifuge, et d'obtenir une protection anti-taches.

12. Procédé selon la revendication 9, 10 ou 11, **caractérisé en ce que** ledit substrat flexible est choisi dans un groupe comprenant : une longueur de tissu ou de cuir ou une feuille de métal, en particulier d'aluminium.

13. Kit comprenant :
- un panneau flexible selon l'une quelconque des revendications 1 à 8;
- au moins un récipient contenant un mélange homogène d'une dispersion de résine aliphatique à base d'eau et de granulés de pierre ou de matière minérale ;
- une colle élastique, exempte de solvants et de composés de ciment.
